

# UNITED STATES PATENT OFFICE.

OLIVER HARRISSON SHAW, OF TOM'S BROOK, VIRGINIA, ASSIGNOR TO H. W. ORNDORF AND CHARLES EDMONDSON, BOTH OF SAME PLACE.

## HARNESS-OIL.

SPECIFICATION forming part of Letters Patent No. 439,607, dated October 28, 1890.

Application filed August 7, 1890. Serial No. 361,357. (No specimens.)

*To all whom it may concern:*

Be it known that I, OLIVER HARRISSON SHAW, a citizen of the United States, residing at Tom's Brook, in the county of Shenandoah 5 and State of Virginia, have invented certain new and useful Improvements in Harness-Oil, of which the following is a specification.

The object of the invention is to produce and supply a superior oil or dressing for use 10 on harness that may be cheaply and readily manufactured and which will keep indefinitely and be effective in use, as will be more fully hereinafter described.

The ingredients of the compound and their 15 proportions are as follows: For one gallon of the oil I preferably use neat's-foot oil, three quarts; beef-tallow, one pound; castile soap, one pound; lamp-black, one-fourth pound; gum-shellac, one-fourth pound; ivory-black, 20 one-fourth pound; gum-arabic, three ounces; rosin, one ounce. The proportion of these ingredients may be varied without departing from the invention.

The ingredients are preferably compound- 25 ed in the following manner: Into a heated kettle or other vessel is introduced the soap,

finely comminuted, together with sufficient water to dissolve the same. The gum-arabic and gum-shellac are then added and stirred until thoroughly dissolved and combined with 30 the soap and water, when the oil, tallow, lamp-black, ivory-black, and rosin are added in the order named. The compound is preferably allowed to remain over the fire about thirty minutes, after which it is put up in cans 35 ready for use.

Having described my invention, what I claim, and desire to secure by Letters Patent, is—

The compound herein described, consisting 40 of the following ingredients in substantially the proportions specified: neat's-foot oil, tallow, soap, lamp-black, gum-shellac, ivory-black, gum-arabic, and rosin, substantially as described. 45

In testimony whereof I affix my signature in presence of two witnesses.

OLIVER HARRISSON SHAW.

Witnesses:

OMER SHIPE,  
M. C. KRONK.